

Nov. 14, 1950

J. L. H. JONKER ET AL

2,530,167

DISCHARGE TUBE

Filed March 1, 1947



JOHAN LODEWIJK HENDRIK JONKER  
& EDUARD GERARDUS DORGELO  
INVENTORS

BY *Jan M. Vugel*

AGENT

## UNITED STATES PATENT OFFICE

2,530,167

## DISCHARGE TUBE

Johan Lodewijk Hendrik Jonker and Eduard Gerardus Dorgelo, Eindhoven, Netherlands, assignors to Hartford National Bank and Trust Company, Hartford, Conn., as trustee

Application March 1, 1947, Serial No. 731,802  
In Belgium December 14, 1944

Section 1, Public Law 690, August 8, 1946  
Patent expires December 14, 1964

8 Claims. (Cl. 250—174)

1

This invention relates to an electric discharge tube the electrode system of which comprises at least one cathode and one anode. The invention is more particularly concerned with the improvement in the thermal radiation properties and the selection of secondary emission properties of electrodes that are not coated with primarily emitting substances. Further the invention relates to a method of coating an electrode with a layer possessed of the properties referred to.

It is an established fact that in discharge tubes of the aforesaid kind all the electrodes assume a higher temperature than they have when the tube is put into use under normal conditions. This heating is due both to the normal thermal radiation of the cathode and to the constant bombardment by electrons. Once an electrode has assumed a given temperature it may in turn also heat the adjacent electrodes by radiation. As a matter of course, this heating is greatest in tubes operating with heavy currents, such as transmission valves.

The effects of the heating of the various electrodes are of two kinds. Firstly, the mechanical strength of almost all of the usual materials decreases at an increased temperature. Secondly, the secondary emission factor increases with the temperature. The former fact is always detrimental while the latter may or may not be an adverse factor depending upon the purpose for which the device is designed. Accordingly, precautions have previously been suggested to obviate these difficulties.

These precautions can be divided into two groups, to wit: into those operative to prevent the cause, that is to say excessive heating, and those operative to remove the effects or else to check them.

The second group includes for example the selection of materials refractory to a higher extent and of materials having a low secondary emission coefficient. The invention is however concerned with precautions pertaining to the first group.

It is known that the rise in temperature can be retarded by the use of artificial cooling, for example by a flow of liquid, by the use of cooling fins and by coating the surface of the pertinent electrodes with a substance that improves the thermal radiation. It has previously been suggested to constitute the coating by a thin layer of carbon, for example in the form of soot, or else a layer of a black oxide or an oxide in a black form, for example titanium oxide may be utilized. As the secondary emission generally

2

decreases at lower temperatures, it will fall due to the improved thermal radiation of the electrodes and the consequent lower temperature thereof; most of the aforementioned good radiating substances, particularly carbon, however, also have a low secondary emission factor so that the secondary emission is likewise reduced materially. To sum up the matter shortly it can therefore be established that coating an electrode with a good heat radiating substance generally results in a decrease of the secondary emission. In some cases however, it is desirable that whilst increasing the radiation of an electrode, so that by means of the consequent fall in temperature the mechanical strain on the electrode material may be lessened, the secondary emission be maintained, or else not nullified entirely and in some cases may even be desirable to increase it. The invention has for its object to ensure this proposed purpose.

An electric discharge tube according to the invention comprises a primarily emitting cathode and one or more other electrodes, one of which at least is coated entirely or in part with a mixture of a good heat radiating material and a substance the secondary emission coefficient of which equals or exceeds 1.

Apart from the fact that the temperature of the coated electrodes, in spite of a high load of the tube, remains so low that there is no risk of undue alterations in the functions of the electrodes, for example due to changes in the position relatively to the other electrodes, the invention has the important advantage that the secondary emission can be imparted a given value by the choice of a suitable substance. This is particularly important in connection with those electrodes which while the tube is in use must preferably not take up current, for example control grids. As is well-known, considerable damping is set up in a tuned circuit connected to a control grid, if current from the grid has to be conducted away through the circuit. Now, it is possible for the secondary emission of the electrodes concerned to be such that the current from the electrodes is equal to zero or if desired is even negative.

It is already known to cause the current passing to a grid to be equal to zero by the use of secondarily emitting substances. It was however hitherto impossible to improve the thermal radiation of an electrode by a coating of the surface whilst at the same time imparting a given value to the secondary emission.

Further it is known to coat an electrode of an

electric discharge tube for the purpose of improving the thermal radiation with a layer of carbon, the carbon layer and the electrode being separated by a layer made up of silicates or oxides of beryllium, magnesium or aluminium. This layer prevents the detrimental absorption of the carbon in the electrode but no question of a mixture of carbon and the silicates or oxides arises. The secondary emission of such an electrode will accordingly be practically entirely governed by the carbon layer, the oxide or silicate layer not being on the surface.

It is only natural that the phenomena of grid current, secondary emission, high mechanical strain, and so forth more readily occur with tubes operating with high voltages, for example, transmission valves, so that the invention is particularly useful in connection with tubes of this kind.

In a tube according to the invention the good heat radiating substance may be carbon, for example in the form of soot or of black oxides or oxides in a black form due to grain roughness, for example titanium oxide, zirconium oxide, tungsten oxide, molybdenum oxide, this substance being mixed with the good secondarily emitting substance, which may be constituted, for example, by magnesia, because this is known to have a good secondary emission coefficient and to be secure against high temperatures. Another substance that may be used to obtain good secondary emission is beryllium oxide. The black substance and the good emitting substance are mixed together, for example applied from a suspension to the surface of the electrode, the suspension agent being then removed for example by heating the electrode. The choice of the ratio between the two substances permits of ensuring a given secondary emission factor within certain limits.

In view of an accurate control of the heat radiating and secondary emission properties part of the electrodes may be left uncoated or may be coated merely with secondarily emitting material or merely with thermal radiating substance.

What we claim is:

1. An electric discharge tube comprising a pri-

5  
10  
15

4  
15  
20  
25  
30  
35

marily emitting cathode and at least one other electrode coated with a mixture of a good heat radiating material and a substance the secondary emission coefficient of which equals at least 1.

2. An electric discharge tube as claimed in claim 1, wherein the good heat radiating substance is constituted by carbon.

3. An electric discharge tube, as claimed in claim 1, wherein the good heat radiating substance is constituted by a black metal oxide.

4. An electric discharge tube, as claimed in claim 1, wherein the good heat radiating substance is constituted by a metal oxide in a black form.

5. An electric discharge system as claimed in claim 1, wherein the good heat radiating substance is constituted by titanium oxide.

6. An electric discharge tube as claimed in claim 1, wherein the substance the secondary emission coefficient of which exceeds 1 is formed by oxides of the group consisting of magnesium and beryllium.

7. An electric discharge tube as claimed in claim 1 wherein the substance whose secondary emission coefficient exceeds 1 is magnesia.

8. An electric discharge tube comprising a primarily emitting cathode and at least one other electrode coated with an intimate, uniform mixture of soot and magnesia.

JOHAN LODEWIJK HENDRIK JONKER.  
EDUARD GERARDUS DORGELO.

#### REFERENCES CITED

The following references are of record in the file of this patent:

#### UNITED STATES PATENTS

| Number    | Name                 | Date          |
|-----------|----------------------|---------------|
| 2,012,339 | Edwards et al. ----- | Aug. 27, 1935 |
| 2,233,917 | De Boer et al. ----- | Mar. 4, 1941  |

#### FOREIGN PATENTS

| Number  | Country             | Date           |
|---------|---------------------|----------------|
| 473,398 | Great Britain ----- | Oct. 12, 1937  |
| 492,025 | Great Britain ----- | Sept. 13, 1938 |